

C. N. FORREST,  
ELASTIC BITUMINOUS SPACING PLANK FOR PAVEMENTS,  
APPLICATION FILED JUNE 6, 1913.

1,207,524.

Patented Dec. 5, 1916.

FIG. I



FIG. II



Inventor  
Charles N. Forrest,

By Tracy & Paul,

Attorneys

<sup>Witnesses</sup>  
John G. Berger.  
James H. Bell.

# UNITED STATES PATENT OFFICE.

CHARLES N. FORREST, OF RAHWAY, NEW JERSEY, ASSIGNOR TO THE BARBER ASPHALT  
PAVING COMPANY, OF PHILADELPHIA, PENNSYLVANIA, A CORPORATION OF WEST  
VIRGINIA.

## ELASTIC BITUMINOUS SPACING-PLANK FOR PAVEMENTS.

1,207,524.

Specification of Letters Patent.

Patented Dec. 5, 1916.

Application filed June 6, 1913. Serial No. 772,039.

*To all whom it may concern:*

Be it known that I, CHARLES N. FORREST, of Rahway, in the county of Union and State of New Jersey, have invented certain new and useful Improvements in Elastic Bituminous Spacing-Planks for Pavements, of which the following is a specification, reference being had to the accompanying drawings.

10 My invention relates to the production of a spacing plank of elastic material, which is used as a substitute for and improvement upon the present method of constructing elastic spacing joints or filling blocks as 15 used for the purpose of taking up the expansion and contraction of pavements.

My invention is particularly applicable to block pavements and my spacing planks are designed for use in the same situation 20 and as substitutes for the elastic joints which have been heretofore provided.

In the accompanying drawings, Figure I, represents a spacing plank constructed according to my invention. Fig. II, is a view 25 of a pavement showing the spacing planks in place.

Heretofore the practice in laying paving blocks, such as vitrified brick or wood blocks, has been to place a wooden plank 30 of suitable thickness and length adjacent to the curb on each side of the roadway, and to start and stop the various transverse courses of paving blocks from and ending at such planks, rather than from the curb 35 line proper, or merely by leaving a longitudinal open space adjacent to the curb lines. After a convenient area of blocks have been thus laid, the said strips of wood are removed and the open space from which 40 they have been removed is filled with melted pitch or asphaltum. The object of the filled space thus provided is to allow transverse movement of the paving blocks through expansion by heat or moisture, without dislocation of the curb line or buckling of the 45 road way. I have invented an improved plank for laying such block pavements which obviates the necessity of, first, the employment of the aforementioned wood 50 strips and the danger of disturbing the abutting blocks when that is removed, second, the necessity of melting pitch or asphaltum filler on the street and handling the same in a highly heated and dangerous condition.

Third, the waste of filling material by slopping it about in a fluid condition, and fourth, the production of cleaner and more workmanlike piece of finished pavement. It is obvious that the bituminous planks used for this purpose must be elastic and yielding in order to move in sympathy with the expansion and contraction of the pavement. Also notwithstanding their elasticity or plasticity, they must be sufficiently cohesive and hard under all conditions of atmospheric temperatures to cause individual planks to retain their identity and shape, without sticking or flowing together, during transit from the point of manufacture to the point of use. They must also be sufficiently firm or cohesive to permit of convenient handling and placing. According to my invention, spacing planks fulfilling these requirements are cast from a heated and melted material, in molds of suitable size, say 75 one inch thick, three inches wide and six feet long, but obviously the dimensions may vary to suit different types of pavement or different situations of use.

A suitable bituminous compound for the planks is one consisting of grahamite 21%, petroleum paraffin residuum 49% and 30% of maltha. Such a combination of bituminous substances is characterized by a high melting point, (say over 190° F.) notwithstanding the softness or penetration of the combination, but it is possible by using other hard native bitumens in combination with other bituminous materials to secure this desired relationship between melting point 85 and penetration whereby there is secured a compound which is not hard or brittle at winter temperatures and which will not flow at summer temperatures and which at the same time does not present an excessively 90 sticky surface. Previous efforts to attain this end have not produced the desired combination of qualities, and an envelop or container has been required to render the material transportable. Such a plank is shown 100 at 1, in Fig. I. If made in accordance with the above directions it possesses the required qualities of elasticity, with some plasticity, also of cohesiveness and non-ductility. In Fig. II, I have indicated a portion of a block 105 pavement, showing such planks, 1, 1, inserted adjacent to the curb line 2, 2. Similar transverse spacing planks 3, 3, are also

shown at intervals in this figure. It will of course be understood that these planks may be inserted at any point where it is desired to create an elastic joint in the pavement.

5 It will also be understood that the invention is not limited to a block pavement, nor to the precise dimensions specified.

Having thus described my invention, I claim:

10 A transportable bituminous spacing plank, for use in the formation of joints of pavements comprising a hard native bitumen, petroleum residuum and a heavy viscous bitumen, combined in such proportions

as to produce a substance having moderate 15 penetration, a melting point over 190° F. and that absence of stickiness upon its surface which renders the article capable of transportation and placing without any container.

20 In testimony whereof, I have hereunto signed my name at Maurer, N. J. this 27th day of May, 1913.

CHARLES N. FORREST.

Witnesses:

M. A. BRAM,  
M. Y. GREENLAW.